

April 4, 1939.

G. LIEBMANN

2,152,809

METHOD OF PRODUCING FINELY DIVIDED METALLIC LAYERS

Original Filed May 28, 1935



*F'ig. 1*



*F'ig. 2*



*F'ig. 3*



*F'ig. 4*

Inventor:

*Richard Liebmann.*

## UNITED STATES PATENT OFFICE

2,152,809

## METHOD OF PRODUCING FINELY DIVIDED METALLIC LAYERS

Gerhard Liebmann, Berlin, Germany

Original application May 28, 1935, Serial No. 23,845. Divided and this application December 21, 1935, Serial No. 55,633. In Germany May 31, 1934

2 Claims. (Cl. 250—27.5)

The present invention relates to a transmitter valve for television purposes with a mosaic electrode and methods for producing such a mosaic electrode by forming metallic layers on insulating materials, such, for example, as mica, or the like, whereby the metallic layer consists of the finest particles, which are insulated against each other, and represents in a manner of speaking a mosaic screen composed of single particles of metal. A screen of this nature may be employed more particularly in certain television image recording methods. After corresponding treatment the mosaic screen represents a surface collection of elementary photo-cells, which produce electrical charges corresponding with the particular exposure. These charges may then further be employed for controlling the transmitter in suitable fashion, by transmitting capacitatively these charges to the silvered rear side connected with an amplifier device. This application is a division of application Serial Number 23,845 filed May 28, 1935, and now Patent Number 2,131,187.

The production of the layer consisting of finest particles of metal is accompanied by considerable difficulties, both as regards selection of the material for the intermediate insulating layer as well as the method of insulation.

It is possible to employ mica for the intermediate insulating layer. The use of this material when employing a heating process for dividing a metallic layer into single elementary parts is confronted by difficulties owing to the inconstancy of the temperature and the nature of the surface. When employing a method for producing the distribution by means of engraving machines or in the case of chemical treatment it is impossible in numerous cases, owing to the small powers of adhesion, to produce a metallic layer in corresponding distribution.

According to the invention, there are employed as intermediate dielectric layers sheets of mica or other suitable bases, for example, ceramic material, certain kinds of glass, etc., the surface of this base preferably being made smooth by polishing. On this base there is produced in suitable fashion a metallic coating, for example a silver, copper or the like coating. A metallic coating of this nature may be produced, for example, chemically, by cathode atomization or by thermal application in vapour form. The metallized plates are then heated to high temperature in an atmosphere of indifferent gas or in vacuum. If the metallic coating is of certain thickness (no longer transparent), the temperatures require to

be very high, for example in the case of silver to about 1000°, in order to obtain a brief fusing of the layer of silver, whereby the surface is then converted from the previously unitary structureless metallic surface into a very even mosaic consisting of small drops of metal of negligible diameter and insulated against each other. According to the invention, this heating is performed extremely rapidly, preferably by means of eddy current heating in high-frequency furnaces. In this connection the metallic coating is acted upon not directly, but indirectly by radiation from a heating plate. In the case of very thin metallic layers it is possible to manage with considerably lower temperatures, which in view of the low temperature constancy of mica is of advantage when employing a material of this kind. When using other materials, such as ceramic substances, glass or the like, the surface of the base is preferably made smooth by polishing, in order to accelerate the insular formation during the heating process.

According to the invention, it is also possible to deposit the metallic layer on a heated base, so that small globules are likewise formed right from the commencement. When using mica, however, the method of subsequently heating the deposited metal as described in the above is to be preferred.

An additional method for insular formation resides according to the invention in the fact that a thin layer of silver deposited, for example, on mica is alternately oxidized and reduced. This method is performed in the most convenient form by glow discharge in an atmosphere of alternately introduced oxygen and hydrogen at suitable pressure (approximately 1 mm. mercury). The alternate oxidation and reduction might also be replaced to a certain extent by a suitable temperature treatment. In this connection the silvered plate is heated in oxygen at first up to the temperature for formation of silver oxide, and then additionally heated in vacuum until the silver oxide has become dissociated. The temperature is thereupon again lowered, etc. In the case of the glow discharge method the silver layer to be granulated is in the most convenient form placed opposite to a plate connected up as anode, with the intermediate connection of a grid-like electrode connected up as cathode. In this respect the layer of silver does not possess any electrically conductive connection with the cathode. The layer of silver might also be connected up as cathode. In this, however, there has been found to exist the dis-

advantage that the oxidizing and reducing process takes place more strongly in the vicinity of the connection between the lead and the layer than at other points. As final stage of the process, after production of the discrete particles of silver, there is conveniently performed a light oxidation, as in this manner it is possible to obtain a layer which is advantageously suited for photo sensitization.

10 In the drawing there is shown diagrammatically by way of example the arrangement for carrying out the method according to the invention. In the drawing—

Fig. 1 shows the indirect heating by means of a heating plate 1, which heats by radiation the layer of silver 2 mounted on the supporting material 3, for example mica. Since this heating required to commence instantaneously, the heating is preferably performed by eddy currents, 20 which is represented diagrammatically by the high-frequency coil 4.

Fig. 2 shows the arrangement for carrying out the glow discharge process. In the same there is provided an electrode 5, which is connected up as 25 anode and is situated opposite to a grid-like cathode 6. The metallic layer 7 to be granulated is arranged within reach of the glow discharge which develops in the case of a suitable filling of gas. 7 is the metallic layer on the base 8. In 30 Figs. 3 and 4 there is illustrated by way of example the finished product. In these 9 is the intermediate dielectric layer, which acts as base for the coatings 10 and 11. The coating 10 represents the thin layer of metal divided upon into 35 finest elementary particles, whilst 11 is intended as capacitative counter-coating for the photo-cell arrangement.

The experiments according to the invention have proved especially useful the following special embodiment of the present invention.

40 A well-cleaned mica plate with all grease removed is coated by the thermal vaporization of silver with a silver layer of approximately  $\frac{1}{10}$ — $\frac{1}{100}\mu$  in thickness. A thickness of the layer approximately midway of the stated range, i. e., approximately  $\frac{3}{100}$  to  $\frac{5}{100}\mu$  produced the best results. The application of the layer by vaporization is performed in a suitable vessel from which the air has been removed, the distance between 45 the mica plate to be treated and the evaporation furnace being of such extent that a very even coating is obtained. Insulation edges of a desired kind may be allowed to remain by selective screening. After the application of the silver 50 layer by vaporization has been completed a certain amount of air or oxygen is allowed to enter the vessel, and the part of the vessel in which the plate is situated, is heated to approximately 400—450° C. This latter operation extends over 55 a period of approximately 15 to 30 minutes.

After cooling it will be noticed that the coating on the plate has been divided into single well-separated crystals of about  $1\mu$  in size.

It has been found that to obtain this effect it is necessary

1. To adhere to the above stated range as regards the thickness of the layer, and

2. To employ a suitable gas atmosphere.

If the initial layer is made thinner, a "granulation" of any kind is not to be determined with 10 the usual optical means available. If the layer is too thick, there is certainly a granulation up to a certain point, but the particles are situated so close together that the requisite insulation may be not obtained. If on the other hand the 15 layer is still thicker (completely opaque), a distribution according to the described process may not be accomplished at all. In this case temperatures would require to be employed which come very near to the fusing point of the silver 20 (800 to 1,000° C.), and considerable difficulties are then encountered in preventing the mica from becoming entirely useless. The size of the formed particles is also a wholly different one in the last 25 mentioned case. Further, it has been found that even with suitable layers a separation does not take place when the process is performed in an extremely high vacuum (higher than  $10^{-5}$  mm. Hg). The presence of a certain gas atmosphere 30 (presumably oxygen) is accordingly necessary for the separation at the low temperature stated.

Mica plates of this kind, which are furnished with a silver screen in the manner stated, may then be employed in the known fashion, by silvering the rear side and by oxidation and sensitization of the front screen surface, as light-sensitive 35 mosaic electrodes in television transmission tubes, for instance, tubes known under the name of "Iconoscope."

I claim:

1. In the process of manufacturing a photoelectric mosaic screen for television transmission tubes, the steps of coating a thin mica plate by thermal vaporisation of silver in vacuum with a transparent silver layer of approximately  $-\frac{5}{100}$  micron in thickness, and of granulating this 45 layer into fine areas by heating the plate in a rarified atmosphere containing oxygen to a temperature below 500° C.

2. In the process of manufacturing a photoelectric mosaic screen for television transmission tubes, the steps of coating a thin mica plate by thermal vaporisation of silver in vacuum with a transparent silver layer of approximately  $-\frac{5}{100}$  micron in thickness, and of granulating this 55 layer into fine areas by heating the plate in a gas atmosphere of about 1 mm. mercury pressure during 15 to 30 minutes to a temperature below 500° C.

GERHARD LIEBMANN. 60